

Oct. 8, 1935.

E. H. BUCY

2,016,314

CRYSTAL LACQUER COATING AND METHOD OF MAKING SAME

Filed Oct. 14, 1933



Fig. 1.



Fig. 2.

EDMOND H. BUCY, <sup>Inventor</sup>

By *Samuel Henick*,  
<sup>Attorney</sup>

## UNITED STATES PATENT OFFICE

2,016,314

CRYSTAL LACQUER COATING AND METHOD  
OF MAKING SAMEEdmond H. Bucy, Waukegan, Ill., assignor to  
Atlas Powder Company, Wilmington, Del., a  
corporation of Delaware

Application October 14, 1933, Serial No. 693,656

1 Claim. (Cl. 91—68)

This invention relates to coatings for all kinds of surfaces and the invention particularly relates to improved surface coatings of the frosted or crystal type, the object of the invention being 5 to provide surfaces presenting frosted or crystalline structures of greater durability and beauty than those heretofore known.

Surface coverings of the crystal lacquer type have been known for a considerable number of 10 years, I have found that crystal lacquer films, for instance, such as made by the process described by Ossian Rosquist in his application, Serial No. 276,799, filed May 10, 1928, entitled "Liquid coating composition and film embodying crystalline 15 structures", or by the process described by Rieder, German Patent No. 266,265, October 20, 1913, are not resistant enough to friction at those particular spots where the crystalline substance, embodied in such liquid coating compositions, upon 20 the drying of the lacquer separates out in crystalline form and usually is covered with an extremely fine film of lacquer.

It requires extreme care in the application of 25 these liquid coating compositions to obtain smooth surfaces, and the time spent in applying such compositions and in such manner as to obtain smooth surfaces, is very often wasted because the film is not sufficiently resistant to friction. A very slight scratch is sufficient to mar the beauty 30 of the film, for the scratch bares the crystalline substance and with each wiping new particles of the crystalline substance are broken off and carried along by the wiping cloth so that the surface is soon dulled by the fine particles of the crystalline substance.

It is, therefore, the primary object of this invention to provide a crystal lacquer coating sufficiently resistant in the effects noted, together with a process by which smooth surfaces may be 40 readily obtained in an economical manner.

It is another object of the invention to provide 45 a crystal lacquer coating which may be applied to all objects, particularly those having smooth surfaces, such as glass, metals, paper and any other material, including those of wood, the pores of which have been filled in any of the ways known to the art.

It is also an object of the present invention to 50 provide a crystal lacquer coating which may be finished or toned in any color and in which the size of the crystals may be regulated.

It depends on the kind of surface on which the 55 crystal lacquer coating is to be applied as to whether or not the surface should first be provided with a priming or under-coat. Since wood is rather porous, it should be treated first with a priming coat to seal the pores. It is, of course, to be understood that this priming coat can vary considerably as to its composition and color. It 60 suffices to say that any priming coat, whether it

be an oil, shellac, or lacquer containing either cellulose ester, such as nitro-cellulose, acetyl-cellulose, or cellulose-ether, such as methyl-cellulose, ethyl-cellulose, baked enamel, or an aqueous suspension of any pigment filler or similar composition, will be of service, provided it fills the pores of the wood, pasteboard, or other surface, in the desired way. Likewise metals may first require a priming coat since various cellulose derivatives, forming the body of the lacquer, 10 may not adhere enough to the blank metal sheet. If any such priming coat is deemed necessary, any suitable priming coat known to the art, may be applied to the metal surface.

The invention will be fully understood from 15 the following description and from the accompanying drawing, which illustrates a surface provided with my new crystal lacquer coating and in which parts are broken away to fully disclose the individual layers of the coating.

Figure 1 discloses the material applied to a 20 wood base and

Figure 2 discloses the material applied to a metal base.

Referring to the drawing the numeral 1 denotes a priming or under-coat first applied to the 25 surface A. This under-coat, or a plurality of the same, should suitably consist of a composition, which will readily dry and harden, so as not to cause any delay, for which reason I elect cellulose acetate as an example of the many possible materials suitable for this purpose. This coat 1 may have any desired coloring or toning matter.

Over this priming or under-coat 1, I apply a 30 coating 2 constituting the crystal lacquer composition which comprises a suitable lacquer base with crystalline compounds dissolved therein. Examples of suitable crystalline compounds are naphthalene, anthracene and other suitable crystalline substances, mostly of organic origin. 35 The following is an example of a composition 40 constituting a crystal lacquer suitable for the purposes stated.

|                    | Parts |
|--------------------|-------|
| Naphthalene        | 10 45 |
| Ester gum          | 5     |
| Toluene            | 15    |
| Ethyl-oxy-butyrate | 40    |
| Cellulose nitrate  | 5     |
| Acetone            | 25 50 |
|                    | 100   |

In due time, upon the reduction of the quantity 55 of the solvent by evaporation, the naphthalene crystallizes out and upon the further evaporation of the solvent the crystals of the naphthalene are embedded in the gradually forming film of cellulose ester and of the ester gum. It is, of course, possible to regulate the size and eventu- 60

ally also the system of the crystals according to desire by varying the quantity of the solvent and the rate of evaporation. The crystal lacquer coat 2, obtained by the aforesaid operations, is not colored or toned, so as not to affect the beauty of the crystals embedded therein.

It is indeed one of the essential features of my invention that care be taken not to mar in any respect the structure of the crystals and thus detract from the beauty of the same.

In accordance with this intention I next apply over the dry crystal lacquer coat, a stop-off coat 3, comprising an aqueous solution of any adhesive or substance, which upon drying leaves a lustrous skin, or glaze. Such substances are, for instance, animal or vegetable glues, casein and inorganic substances, such as alkali-metal silicates, particularly sodium silicate, and water soluble cellulose ethers, such as methyl-cellulose or ethyl-cellulose. The aqueous solution of the stop-off coat 3 should be a very dilute one and preferably should be practically colorless. Ordinary casein dissolved in slightly alkaline water, or ammonia water, gives good results.

The effect obtained by this transparent stop-off coat is one of a peculiar kind in that the fine crystals, which have been formed in the crystal lacquer are preserved and on account of the light reflections are beautifully set off against each other; the effect of this stop-off coat can be compared, so to say, to the effect accomplished by the

oil immersion in microscopic work. No coloring or toning material interferes with their appearance and as the water soluble or stop-off coat prevents the next following top coat 4 from dissolving away the crystals, the beauty of the crystals is fully preserved.

The top coat 4, or a plurality of the same, may consist of any cellulose lacquer or varnish; the last layer of the coat 4 may be polished or may be left untouched, if desired.

Having described my invention, what I claim is:

The herein described method of surface ornamentation which comprises coating an article with a water insoluble lacquer containing a substantially water-insoluble crystalline substance of such nature that upon drying said crystalline substance takes the form of a multiplicity of individual crystals of a determined pattern, applying thereto after drying a stop-off coat of an aqueous material yielding a transparent film, and applying over the last named coating a coating of a non-aqueous material yielding a transparent waterproof top coat, the water insoluble nature of the lacquer, the aqueous nature of the stop-off coat, and the non-aqueous nature of the top coat rendering the lacquer coat insoluble in the stop-off coat and rendering the stop-off coat insoluble in the top coat.

EDMOND H. BUCY.